

## UNITED STATES PATENT OFFICE.

HENRY C. KIRK, OF ROLAND PARK, AND GEORGE H. DUMLER, OF BALTIMORE,  
MARYLAND.

## ALLOY.

Application filed March 5, 1921. Serial No. 450,011.

*To all whom it may concern:*

Be it known that we, HENRY C. KIRK and GEORGE H. DUMLER, citizens of the United States of America, the former residing at Roland Park, Baltimore County, Maryland, and the latter in the city of Baltimore, State of Maryland, have invented certain new and useful Improvements in Alloys, of which the following is a specification.

The metal which is the subject of this invention in its preferred form is an alloy of copper containing approximately 10% iron. The applicants have made extensive investigation on the subject of copper and iron alloys. Such alloys were prior to these experiments by these applicants, so difficult of production that they were unknown in the industries. As a result of their experiments the applicants have discovered that nickel in comparatively small quantities can be used as a vehicle causing copper to alloy with iron. It is found that approximately 1% of nickel is sufficient to introduce into and to cause to alloy with copper at least 10% of iron producing an alloy of 10% iron, 1% nickel, the balance being copper.

An alloy has however been made in proportions varying from 3 to 20% iron, nickel being used as a vehicle for the iron, preferably in the proportion of one part nickel to 3 to 12 parts iron, the remainder of the alloy being copper.

The resulting alloy has a tensile strength of from 59,000 to 61,000 lbs. per sq. in. when rolled and annealed and an elastic limit of 14 to 16% in two inches. The metal is intended to be used as a substitute for brass to which it is superior, in strength, and in the

fact that it can be hot rolled whereas brass cannot. Also it does not require overhauling, i. e., it casts clean, has a high melting point and produces good sand castings for valves and the like. Also it has greater non-corrosive qualities than has brass or any similar alloy or mixture.

The simplest method of making the alloy out of common commercial materials is by dissolving iron in a molten mixture of nickel and copper preferably near the melting point of the mixture which is closely related to the melting point of nickel, the nickel having a solvent effect on the iron which alone, has a higher melting point than nickel.

We have thus described specifically and in detail two alloys embodying our invention. In order that the nature of the same may be clearly understood the specific terms herein are used descriptively rather than in a limiting sense, the scope of the invention being defined in the claims.

What we claim and desire to secure by Letters Patent is:

1. A copper alloy substantially in the proportions of 10% iron, 1% nickel, the balance being copper.
2. An alloy consisting in the main of copper and containing from 3 to 20% iron and a small quantity of nickel in the proportion of 1 part nickel to 4 to 12 parts iron.

Signed by us at Baltimore, Maryland, this 2nd day of March, 1921.

HENRY C. KIRK.  
GEORGE H. DUMLER.

Witnesses:

PORTER H. FLAUTT,  
EDWIN F. SAMUELS.